# EUROPEAN PATENT SPECIFICATION

(11) **EP 1 953 280 B1**
(45) Date of publication and mention of the grant of the patent: **19.10.2011**
(21) Application number: 07123777.0
(22) Date of filing: 20.12.2007
(51) Int. Cl.: D03D 15/06

(54) **Process for the production of a fabric made of extra-fine animal fibres which are not industrially weaveable**
Verfahren zur Herstellung eines Gewebes aus extrafeinen Tierfasern, die nicht industriell gewebt werden können
Processus de production d'un tissu à base de fibres animales extra-fines qui ne peuvent pas être tissées industriellement

(30) Priority: 31.01.2007 IT MI20070151
(43) Date of publication of application: 06.08.2008
(73) Proprietor: Geraldini, Jacopo, 20122 Milano (IT)
(72) Inventor: Geraldini, Jacopo, 20122 Milano (IT)
(74) Representative: Mittler, Enrico

(56) References cited:
- EP-A- 1 061 162
- CN-A- 1 450 216
- GB-A- 775 387
- GB-A- 1 068 662
- JP-A- 55 098 936

## Description

The present invention relates to a process for the production of a fabric made of extra fine animal fibres which cannot be women by an industrial machine.

In the field of extra fine animal fibres, it is known that fibre yarns having a very high count may industrially be made, for instance worsted yarns having a count in the range between 200 dtex and 50 dtex. However, it is similarly known that such yarns have a kinetic resistance which is so low as not to allow them to be subjected to an industrial weaving operation, requiring a breaking strength not lower than 80-100 grams.

GB-A-1 068 662 discloses a bulky stretchable yarn of substantially solid structure, for example of silk, which is associated with a substantially unstretchable yarn, for example of wool, to obtain a two-ply yarn around which a binding yarn is helically twisted to form a three-ply yarn.

EP-A- 1 061 162 discloses a process for manufacturing a pure cashmere textile article in which first yarns of pure cashmere fibres are associated by doubling with second yarns of synthetic fibres which are then dissolved after weaving of the doubled yarns.

GB-A-775 387 discloses a process for manufacturing spun yarns in which a yarn is produced by mixing soluble and insoluble fibres.

CN-A-1 450 216 discloses a fabric made of extra fine animal fibres consisting only of blended yarns formed by animal fibres having a count in the range between 200 dtex and 50 dtex.

It is the object of the present invention to provide a process allowing the weaving of yarns made of extra fine animal fibres, specifically cashmere fibres, which otherwise cannot be wormen by industrial machine.

In view of such a purpose, the process according to the present invention is **characterised in that** it comprises the sequence of steps recited in claim 1.

Fabrics made of extra fine animal fibres, specifically cashmere fibres, which up to now could not be subjected to industrial weaving, may be obtained industrially in this manner.

Blended yarns (or so-called "intimate blend yarns") indeed allow to achieve incredibly high counts by mixing very soft though very low tenacity short fibres, such as extra fine cashmere fibres, with extremely fine and very high tenacity long fibres, such as silk.

An appropriate percentage of the two kinds of fibres is 80% cashmere (WS) and 20% silk (SE).

The doubling is with carried out with yarns having substantially the same count and with a torsion in the direction opposite to that of the blended yarns. The torsion of the single yarns is of the Z type and the doubling torsion is of the S type.

An extremely soft and together resistant fabric is the result of the doubling torsion in a direction opposite to that of the blended yarns, even though extra fine animal fibres which are not otherwise industrially weaveable have been used.

An examplary embodiment of the process according to the present invention will now be described in detail with reference to the accompanying drawings, in which:
Figure 1 shows a blended yarn made of extra fine cashmere fibres and silk fibres, doubled with a yarn made of synthetic polyvinyl fibres soluble in a slightly acidic solution at a high temperature;
figure 2 shows a portion of a coarse fabric obtained by weaving of doubled yarns such as those in figure 1;
figure 3 shows the same portion of fabric after dissolving the yarns of synthetic fibres.

A blended yarn 1 formed by 80%WS - 20%SE with an extra fine 66 dtex count is considered here by way of example. The yarn 1 has been made by traditional spinning with a Z torsion of 1100 rounds/linear meter.

The blended yarn 1 is then doubled with a yarn 2 having a substantially equivalent count, and a Z torsion of 1000 rounds/linear meter, consisting of synthetic (so-called "water-soluble") polyvinyl fibres (PVA). These fibres can be dissolved in a slightly acidic aqueous solution at a high temperature. The yarn 2 may be made of spun fibres with a cotton cut (thus having a discontinuous nature).

The doubling is carried out with a S torsion of 440 rounds/linear meter, so as to obtain a correct final balancing of the doubled yarn.

The resulting doubled yarn, indicated by numeral 3 in figure 1, is obviously made of 50%PVA, 40%WS and 10%SE.

As shown in figure 2, an appropriate number of doubled yarns 3 is subsequently subjected to a traditional warp and weft weaving (or weaving on a circular Jersey type machine), in which the polyvinyl yarns 2 serve as a support to allow the weaving of the blended yarns 1, which are otherwise not industrially weaveable.

The coarse fabric thus obtained, which may have any cloth, twill or jacquard-type weave, clearly has the same composition as the doubled yarn 3.

Such a coarse fabric is then subjected to a scouring dyeing step, during which it is dipped in an aqueous solution of about 50 litres per kg of polyvinyl with a slightly acidic pH (about 4,5) at a temperature between 30°C and 100°C (depending on the nature of the PVA yarn).

The PVA yarn 2 is thus eliminated by dissolution or melting, leaving a final fabric (fig. 3) consisting exclusively of blended yarns 1 and therefore having a final composition of 80%WS - 20%SE with a 66 dtex count, which is impossible to achieve industrially by traditional techniques.

In virtue of the doubling S torsion in a direction opposite to that of the single yarns 1 and 2, after the melting of the PVA yarns 2, the remaining yarn 1 has a torsion which is equivalent to the sum of the spinning torsion (1100 Z) and the doubling torsion (440 S), that is in the example considered equivalent to 660 Z. In virtue of this reduced torsion the resulting fabric is therefore extremely soft, as well as having an extra fine count.

Finally, with the process according to the present invention a fabric may be made having the following unique properties:
a) it is formed by a yarn having an extra fine count which would not otherwise be industrially woven;
b) it is extremely soft.

## Claims

1. A process for the production of a fabric made of extra fine animal fibres which cannot be woven by an industrial machine, **characterised in that** it comprises the following sequence of steps:
a) spinning of blended yarns (1) formed by 80% cashmere animal fibres having a count in the range between 200 dtex and 50 dtex and by 20% silk fibres, the blended yarns (1) having a Z twist of 1100 rounds/linear meter;
b) doubling of each of said blended yarns (1) with a corresponding synthetic yarn (2) made of PVA synthetic fibres soluble in a liquid solution having a PH of about 4.5 at a temperature between 30°C and 100°C, the synthetic fibres (2) having substantially the same count as the blended yarns (1) and a Z twist of 1000 rounds/linear meter, doubling being carried out with S torsion of 440 rounds/linear meter;
c) weaving of the doubled yarns (3);
d) dissolving said synthetic fibre yarns (2) by means of a liquid solution having a PH of about 4.5 at a temperature between 30°C and 100°C.

## Patentansprüche

1. Verfahren zur Herstellung eines Gewebes, aus extra feinen Tierfasern, die mit einer Industriemaschine nicht gewebt werden können, **dadurch gekennzeichnet, dass** das Verfahren die folgende Schrittfolge aufweiset:
a) Spinnen von gemischten Garnen (1), welche von 80 % tierischen Kaschmirfasern mit einer Dichte im Bereich zwischen 200 dtex und 50 dtex und von 20% Seidenfasern gebildet werden, wobei die gemischten Garne (1) eine Z-Drehung von 1100 Drehungen/Linearmeter haben;
b) Doublieren der jeweiligen gemischten Garne (1) mit einem entsprechenden synthetischen Garn (2), hergestellt aus synthetischen PVA-Fasern, welche in einer flüssigen Lösung mit einem pH-Wert von etwa 4,5 bei einer Temperatur zwischen etwa 30°C und 100°C löslich sind, wobei die synthetischen Fasern (2) im wesentlichen dieselbe Dichte wie die gemischten Garne (1) und eine Z-Drehung von 1000 Drehungen/Linearmeter haben, und wobei das Doublieren mit einer S-Torsion von 440 Drehungen/Linearmeter erfolgt;
c) Weben der doublierten Garne (3);
d) Auflösen der synthetischen Fasergarne (2) mit Hilfe einer flüssigen Lösung, welche einen pH-Wert von etwa 4,5 hat, bei einer Temperatur zwischen 30°C und 100°C.

## Revendications

1. Procédé pour la production d'un tissu réalisé avec des fibres animales extrafines qui ne peuvent pas être tissées par une machine industrielle, **caractérisé en ce qu'**il comprend la séquence d'étapes suivante :
a) filer des fils mélangés (1) formés par 80 % de fibres animales de cachemire ayant un titre compris entre 200 dtex et 50 dtex et par 20 % de fibres de soie, les fils mélangés (1) ayant une torsion Z de 1100 tours/mètre linéaire ;
b) doubler chacun desdits fils mélangés (1) avec un fil synthétique (2) correspondant réalisé avec des fibres synthétiques de PVA solubles dans une solution liquide ayant un Ph d'environ 4,5 à une température comprise entre 30°C et 100 °C, les fibres synthétiques (2) ayant sensiblement le même titre que les fils mélangés (1) et une torsion Z de 1000 tours/mètre linéaire,
le doublage étant réalisé avec la torsion S de 440 tours/mètre linéaire ;
c) tisser les fils doublés (3) ;
d) dissoudre lesdits fils en fibres synthétiques (2) au moyen d'une solution liquide ayant un Ph d'environ 4,5 à une température comprise 30 °C et 100 °C.
